

E. WEINHEIM.

LEATHERLIKE SURFACED FABRIC AND PROCESS OF MAKING SAME.

APPLICATION FILED OCT. 3, 1908.

926,526.

Patented June 29, 1909.



Witnesses:  
W. L. Wocher  
George Pilschen

Inventor  
*Emil Weinheim.*  
By His Attorney  
*Leonard Day.*

# UNITED STATES PATENT OFFICE.

EMIL WEINHEIM, OF NEW YORK, N. Y.

## LEATHERLIKE SURFACED FABRIC AND PROCESS OF MAKING SAME.

No. 926,526.

Specification of Letters Patent.

Patented June 29, 1909.

Application filed October 3, 1908. Serial No. 455,952.

*To all whom it may concern:*

Be it known that I, EMIL WEINHEIM, a citizen of the United States, and a resident of the borough of Manhattan, county, city, and State of New York, have invented certain new and useful Improvements in Leather-like-Surfaced Fabrics and Processes of Making Same, as set forth in the following specification.

10 This invention relates to a leatherlike surfaced fabric and the process of making the same.

The object of this invention is to form a water resisting finish surface upon a previously prepared commercial fabric such as textile fabric or tough paper supplied in bolts or rolls. The process applies to the manner of treating the fabric preparatory to applying the finish coating; to the manner of 20 applying coating; and to the composition of the coating itself called a patina.

One object of the invention is to employ such a patina that it will thoroughly embody and incorporate itself about and upon the 25 surface fibers of the fabric and may be insolubilized *in situ*, that is, when it has become incorporated with the surface fibers of the fabric, although it was more or less soluble before application.

30 Provision is made for applying an even coating of patina of the desired thickness and for scrubbing it into and over the surface of the fabric.

It is a further object of the invention to 35 provide for the continuous and progressive commercial production of the coated fabric in strips of any desired length rather than in sheets of definite dimensions.

In carrying out the process a solution of 40 dichromate of potassium may first be incorporated in and about the surface fibers of the surface of the strip to be coated with the patina. The strip is then thoroughly dried and the coating of patina of special composition 45 is subsequently applied to the surface impregnated with dichromate of potassium. The patina is rendered insoluble by the dichromate of potassium under the influence of heat and pressure.

50 The above and further objects of the invention will be pointed out in the accompanying claims and will be clear from the following description read in connection with the accompanying drawings which form part 55 of this application and in which the single

figure is a diagrammatic representation of apparatus for carrying out the process.

1 designates a roll of any suitable commercial fabric 2 which may be common drill, other strong textile fabric or tough paper fabric. This fabric may be dyed any desired color or undyed if desired. The fabric is illustrated as first passing between the vertically positioned rolls 3 and 4, of which the doctor roll 4 is shown partially immersed in a solution of dichromate of potassium 5 contained in a suitable trough 6. The roll 4 applies an even coating of the dichromate of potassium solution to the under side of the strip 2. The strip 2 then passes over and under suitably heated drying rolls 7 and 8 where the water in the dichromate solution is dried out leaving a crystalline deposit of dichromate of potassium in and about the fibers of the surface 9 of the strip 2. The surface of the strip thus treated is termed by the applicant a "dichromatized surface." The strip 2 then passes about a large heated cylinder 10 driven independently in the direction of the arrow. Beneath the roll 10 is a suitable tank or trough 11 filled with a suitable patina of the desired color and composition. The preferable composition is what may be termed a leatherfying composition and will subsequently be described. The doctor roll 13 is partially immersed in the patina 12 and is driven independently of the roll 10 in the direction of the arrow. The doctor roll 13 may be adjusted horizontally by the means 14 and it may be adjusted vertically by the means 15. Throughout both its horizontal and vertical adjustment, its movement is parallel to itself and to the axis of large cylinder 10. The vertical adjustment serves to regulate the degree of immersion in the patina of the doctor roll 13 and the consequent thickness of the coat of patina carried by the doctor roll. The horizontal adjustment determines the pressure with which the doctor roll contacts with the strip 2. One or more 100 brushes 16 are positioned so as to contact with the patinated surface 9 of the strip 2 while the strip is still in contact with the large heated cylinder 10. These brushes may be mounted to play in a vertical guide 17 horizontally adjusted by the means 18. The pitman and link 19 and 20, which may suitably be driven, impart an up and down scrubbing motion to the brushes 16 while the horizontal adjusting means 18 may serve to regulate the 110

pressure of the brushes upon the strip 2. The scrubbing of the brushes is back and forth in the direction of the movement of the strip 2.

The strip 2 passes from the heated cylinder 10 and from the brushes 16 to an idler or driven roll 21 thence upon an endless carrier 22 which may be driven at a greater speed than the speed of the cylinder 10 so as effectually to drag along the fabric by frictional 10 contact therewith and to insure its proper progress through the apparatus.

In passing off of carrier 22 the strip 2 is engaged upon suitable horizontal rods 23, 24 and 25, etc., placed across an intermittently 15 driven endless chain 26 suitably supported. The fabric 2 droops down in festoons 27, 28, 29 etc., between the rods 23, 24 and 25, etc. When thus festooned the fabric is subjected to a heated drying atmosphere to dry out the 20 patina.

It is to be understood that the fabric, thus treated by one passage through the apparatus illustrated, may be again treated in the same manner to increase the density of the coating 25 of patina or it may receive a subsequent coating of patina without first being treated with the dichromate of potassium. It is also to be understood that for some purposes the fabric may be treated just as described but with the 30 omission of the initial treatment by dichromate of potassium. It should also be understood that any substance having the equivalent effect of dichromate of potassium upon the patina may be employed in place thereof.

35 A desirable composition for the patina and which is well designated a leatherfying composition may be as follows: 1. Suitable coloring matters, preferably mineral. 2. Viscous animal parts, such as bone glue, 40 glutin and other glutinous matter of animal origin. 3. Vegetable oils, such as palm oil, olive oil and others. 4. Hydro-carbons, such as parafin, vaseline, bitumen or others. 5. Metallic salts, such as hydrated oxid of 45 zinc, potassium, lead and aluminum. 6. Animal fats, such as tallow, suet and others. 7. Suitable saponifying agents, such as sodium and potassium alkalies.

The various ingredients enumerated may 50 be employed in various proportions easily determined by experiment but their various proportions should be such as to render the resultant composition sufficiently fluid at approximately 70 to 80° Fahrenheit for satisfactory application to the strip by means of the doctor roll. Selections from the first six sets of ingredients may be kneaded and mixed together under the influence of heat in a suitable vessel and then one of the seventh 55 set of ingredients added; or if desired various changes in the selection of elements from those enumerated or from their equivalents 60 may be made as desired.

In some instances it may be desirable to 65 heat the patina 12 while in the trough 11 to

keep it fluid although for commercial operation it may be found that the heat from the large cylinder 10 will keep it warm enough. This cylinder 10 should be heated to a considerable temperature upward of 80° Fahrenheit enough to cause the dichromate of potassium to insolubilize the patina but insufficient to injure the fabric passing over same. White light also aids the process.

After a sufficiently homogeneous coating 75 of patina has been applied as described, the strip thus coated may have a coating of varnish applied to the surface to give it the desired luster. The varnish may be applied in an apparatus similar to that shown in the 80 figure but, of course, without the application of dichromate of potassium. A suitable varnish for the purpose may be formed of a solution of casein substances, vegetable oils, fatty acids such as olein or the like, and a 85 suitable saponifying agent.

After the coating of varnish has been thoroughly dried the finish surface of the strip may then be calendered by any suitable calender such as a cylinder calender preferably heated. 90 If desired a final coating of a watery solution of formaldehyde and alcohol may be applied to both the finished surface of the fabric and to the unfinished surface of the fabric or to one or the other only. This treatment with 95 formaldehyde compacts the surface of the product. The fabric should then be redried when it will be found that it is moisture resisting to a large degree and resembles finished leather on its finished surface and in a 100 measure possesses the qualities of leather, of course, within the structural limits of the body fabric employed.

The chief object of this invention is to produce a very cheap product having many desired qualities such as comparative durability and leather like appearance.

When the fabric strip is first treated with dichromate of potassium before the application of the patina, the patina forms a very close 110 union with the fabric and is impervious to moisture and consequently will resist peeling off to a great degree. The fabric with such a finish does not require a coating of varnish or of formaldehyde to render it insoluble or impervious to moisture although such a coating may be employed to add luster to the finish. Insoluble means insoluble in water.

115 Coatings which rely entirely upon varnish coatings to render them impervious to moisture are radically different from the fabric with an insoluble coating which I have described. A surface coating of varnish is more or less subject to cracking and wherever cracked the underlying patina is readily 120 attacked by penetrating moisture.

125 Although a complete description of the steps of this invention has been given, it is to be understood that they may be varied within the general scope of the invention. It is 130

- also to be understood that the apparatus illustrated diagrammatically has been shown merely for the purpose of illustrating means for carrying out the process.
5. What is claimed and what is desired to be secured by United States Letters Patent, is:
1. The process of producing a leatherlike surfaced fabric comprising, continuously passing a continuous strip of artificial fabric 10 through progressive steps,—first coating the surface to be finished with a solution of dichromate of potassium; effecting a deposit of dichromate of potassium by drying out the water in solution; applying an even 15 coating of a patina of more or less soluble leatherfying composition to the said surface; compacting and incorporating said patina onto and into said surface under the influence of heat to insolubilize said patina; and subjecting the coated fabric to a heated drying 20 atmosphere.
  2. The process of producing a leatherlike surfaced fabric comprising, continuously passing a continuous strip of artificial fabric 25 through progressive steps,—first coating the surface to be finished with a solution of dichromate of potassium; effecting a deposit of dichromate of potassium by drying out the water in solution; applying an even coating 30 of patina of more or less soluble leatherfying composition to the said surface; compacting and incorporating said patina onto and into said surface under the influence of heat to insolubilize said patina; and subjecting the coated fabric to a heated drying 35 atmosphere; applying a superposed coat of varnish; and again drying the product.
  3. The process of producing a leatherlike surfaced fabric comprising, the continuous 40 progressive steps,—applying to the surface of the fabric to be finished a coating of patina comprising a saponified, suitably colored leatherfying composition of animal parts and oily matter; incorporating said patina 45 in and upon the surface fibers of said fabric under heat and scrubbing pressure; drying the product under the influence of heat; applying a superposed coat of saponified varnish; redrying; and calendering said patina 50 coated surface.
  4. The process of producing a leatherlike surfaced fabric comprising the continuous progressive steps,—drying a suitable fabric; applying an even coating of patina comprising, mineral coloring matter, viscous animal parts, vegetable oil, animal fat, hydrocarbon, metallic oxid and a saponifying agent; subjecting the coating of patina to a 55 scrubbing pressure under the influence of heat to effect its compacting upon and incorporation with the surface of said fabric; and drying the product under the influence 60 of heat and the atmosphere.
  5. As an article of manufacture a leatherlike surfaced fabric comprising a body of suitable artificial fabric having a dichromatized surface; a closely compacted and incorporated coating of suitable colored patina comprising a saponified mixture of viscous and leatherfying animal parts, vegetable oil, animal fat, hydro-carbon and metallic oxid and insolubilized *in situ* upon the said dichromatized surface. 65
  6. As an article of manufacture a leatherlike surfaced fabric comprising a body of suitable artificial fabric having a dichromatized surface; a closely compacted and incorporated coating of suitably colored patina comprising a saponified mixture of viscous and leatherfying animal parts, vegetable oil, animal fat, hydro-carbon and metallic oxid 70 and insolubilized *in situ* upon said dichromatized surface; and a coating of saponified casein varnish. 75
  7. As an article of manufacture a leatherlike surfaced fabric comprising a body of suitable artificial fabric; a closely compacted and incorporated coating of suitably colored patina comprising a saponified mixture of viscous and leatherfying animal parts, vegetable oil, animal fat, hydro-carbon and metallic oxid; and a saponified coating of saponified casein varnish, the finished fabric having a formaldehyde compacted exterior surface. 80
  8. As an article of manufacture a leatherlike surfaced fabric comprising a body of suitable artificial fabric having a surface impregnation of dichromate of potassium; a suitably colored coating of patina compacted 85 upon said dichromate treated surface and in partial combination with said dichromate; said patina comprising a saponified mixture of viscous animal parts, oily matter and a metallic oxid, said coating of patina being 90 water insoluble throughout. 95
  9. As an article of manufacture a leatherlike surfaced fabric comprising a body of suitable artificial fabric having a surface impregnation of dichromate of potassium; a suitably colored coating of patina compacted 95 upon said dichromate treated surface and in partial combination with said dichromate; said patina comprising a saponified mixture of viscous animal parts, vegetable oil, animal fat, hydro-carbon and a metallic oxid, said coating of patina being 100 water insoluble throughout. 105
- In testimony whereof, I have signed my name to this specification, in the presence of 110 two subscribing witnesses.
- EMIL WEINHEIM.
- Witnesses:
- LEONARD DAY,  
EDSON B. SAMMIS.